

# United States Patent Office

3,367,868  
Patented Feb. 6, 1968

1

3,367,868

## RUST INHIBITED POLY(HEXAFLUOROPROPYLENE OXIDE) OIL COMPOSITIONS

John Tevlin Skehan, Claymont, Del., assignor to E. I. du Pont de Nemours and Company, Wilmington, Del., a corporation of Delaware  
No Drawing. Filed Apr. 1, 1966, Ser. No. 539,314  
9 Claims. (Cl. 252—34.7)

This invention relates to poly(hexafluoropropylene oxide) oils and more particularly to poly(hexafluoropropylene oxide) oil compositions containing perfluoroalkylether acids and corresponding ammonium salts as rust inhibitors.

There is a definite present need for lubricants which will operate at temperatures above 500° F. for long periods. To date, the only lubricants which even remotely approach serviceability under such conditions are certain polymers of hexafluoropropylene-1,2-epoxide, hereinafter referred to as hexafluoropropylene oxide.

The useful poly(hexafluoropropylene oxide) oils are those of the structures



and



in which  $R_f$  is a perfluoroalkyl group having 1 to about 6 carbon atoms. These oils may be tailored, if desired, to operate at temperatures as high as 800° F. They are not affected by either oxygen or moisture at these temperatures. However, rusting of ferrous metals has been encountered at these temperatures. Accordingly, it is desirable to provide inhibitors which prevent rusting of these metals at extreme temperatures.

These oils are also used to prevent rusting of metal parts at ambient temperatures. Many parts or subassemblies of devices, after being manufactured, are filled with these oils and stored until needed, often a considerable period of time. Although poly(hexafluoropropylene oxide) oils are superior to hydrocarbon oils for this use, complete rust prevention is not obtained with these oils alone.

In order to be useful with these oils, a rust inhibitor must possess a number of specific properties. First of all, it must inhibit rust. Furthermore, it must be soluble in and compatible with the oil. The solubility must be sufficient to provide an effective amount of inhibitor in the oil, both at operating temperatures and at ambient temperatures. There must be no separation of the inhibitor from the oil even while the device containing the oil is not in use. The inhibitor itself must also possess a high degree of thermal stability at the temperatures at which the oils are used. An inhibitor which decomposes under operating conditions will lose its effectiveness rapidly. Moreover, the inhibitor should not seriously affect lubricant properties, particularly lubricity, oil viscosity and oil viscosity index. These and other requirements eliminate most, if not all, known rust inhibitors.

It is an object of this invention to provide poly(hexafluoropropylene oxide) oil compositions containing rust inhibitors which considerably reduce or prevent rusting of ferrous metals even at extremely high temperatures. Other objects will become apparent from the following description of this invention.

It has now been discovered that reduced rusting of ferrous metals in the presence of poly(hexafluoropropylene oxide) oils can be obtained by using a poly(hexa-

2

fluoropropylene oxide) oil composition which comprises poly(hexafluoropropylene oxide) oil of the structure



or



where  $n$ ,  $p$  and  $r$  are integers indicating the degree of polymerization and  $R_f$  is a perfluoroalkyl group having 1 to about 6 carbon atoms, said oil having an average molecular weight of at least about 3,000 and a pour point not in excess of about 50° F. and, as rust inhibitor, an effective amount of perfluoroalkylether acid or corresponding ammonium salt of the structure



in which  $m$  is about 7 to 18,  $B$  is H or  $NH_4$  and  $R_f$  is as previously stated.

Poly(hexafluoropropylene oxide) oils of the above structures are extremely stable at elevated temperatures. Those polymers having average molecular weights of at least about 3,000 and pour points not in excess of about 50° F. are quite useful as lubricating oils. Polymers of the type



having an average molecular weight of about 5,500 to 7,000 are preferred. These molecular weight designations are based upon number average molecular weights obtained by the spectroscopic method. The pour point designation is based upon Federal Test Method Standard 791, method 351.

These poly(hexafluoropropylene oxide) oils may be prepared in several ways. Hexafluoropropylene oxide is readily homopolymerized to products of the structure



where  $n$  is 0 or an integer indicating the degree of polymerization, as described in Canadian Patent No. 725,740, issued Jan. 11, 1966. Polymers of the structure



where  $x$  and  $y$  are each 1 to about 4, are prepared by polymerizing hexafluoropropylene oxide in the presence of a ketone of the structure



as described in Canadian Patent No. 707,363, issued Apr. 6, 1965. Polymers of the structure



where  $z$  is 0 to about 5 are prepared by polymerizing hexafluoropropylene oxide in the presence of an acid fluoride of the formula



as described in French Patent No. 1,362,548.

All of the above polymers are readily hydrolyzed in the presence of water to the corresponding acids of the formula



where  $R_f$  is a perfluoroalkyl group having 1 to about 6 carbon atoms. The acids derived from these products

react with elemental fluorine according to the method of British Patent No. 1,000,802 to form



These polymers also dimerize under the influence of ultraviolet light, as described in U.S. Patent No. 3,214,478, to form oils of the formula



The rust inhibitors used in the compositions of this invention are the perfluoroalkyl ether carboxylic acids and corresponding ammonium salts of the structure



in which  $m$  is about 7 to 18, B is H or  $NH_4$  and  $R_f$  is a perfluoroalkyl group having 1 to about 6 carbon atoms. Preferably  $m$  is about 7 to 10 and  $R_f$  is  $CF_3CF_2CF_2-$ . These acids are prepared by hydrolyzing hexafluoro propylene oxide polymers of the structure



as indicated above. The corresponding ammonium salts are prepared by first mixing the acid with a suitable solvent, such as toluene in which the acid partially dissolves and partially disperses in finely divided form. Ammonia gas is then bubbled through the mixture at room temperature. After all of the acid has been neutralized, the solvent is evaporated under vacuum leaving the solid ammonium salt of the acid.

The poly(hexafluoropropylene oxide) oil composition of this invention should contain an effective amount of the acid or ammonium salt as rust inhibitor. By "effective amount" is meant the amount required to produce a useful inhibitor effect for the required service life of the device containing the oil at the operating temperature. The various ferrous metals differ considerably in the amount of rust which will occur and the amount of inhibitor required to prevent it. Furthermore, inhibitor is probably consumed while doing its job, hence increased service life or higher use temperatures will require larger amounts of inhibitor. Accordingly, the exact amount of inhibitor required for specific applications will vary considerably.

In general, the amount of acid or ammonium salt in the oil composition will be in the range of about 0.1 to 2% by weight. So long as at least about 0.1% of inhibitor is present, a significant amount of rust inhibition is obtained. As the amount of inhibitor is increased, a quantitative reduction in rusting is obtained up to a point. More than about 2% of inhibitor seldom produces any significant increase in effect. To prevent rusting over long periods, it is preferable to add about 1 to 2% of the acid or ammonium salt. These rust inhibitors are completely soluble in the poly(hexafluoropropylene oxide) oils in the required amounts.

The following examples, illustrating the novel oil compositions of this invention and their utility, are given without any intention that the invention be limited thereto. All percentages are by weight.

#### Examples 1 and 2

Oil compositions containing poly(hexafluoropropylene oxide) of the formula



having an average molecular weight of 4,300 and 0.2% of an acid or ammonium salt of the structure



in which B is H or  $NH_4$  are tested for rust preventing qualities using test method D-665 of the American Society for Testing Materials. Procedure B is followed using synthetic sea water. Briefly, the test consists of immersing an iron billet in a mixture of the oil composition and the

sea water for 48 hours, and then examining the surface of the billet for rust.

For comparison, a control experiment in which no inhibitor is present is carried out. The following results are obtained.

TABLE

| Example | Inhibitor     | Percent of Surface Rusted |
|---------|---------------|---------------------------|
| 1       | Acid          | 1                         |
| 2       | Ammonium salt | 0                         |
| Control | None          | 45                        |

#### Examples 3 and 4

Examples 1 and 2 are repeated except that the poly(hexafluoropropylene oxide) oil is of the structure



and has an average molecular weight of 6,200. Similar results are obtained.

Although the invention has been described and exemplified by way of specific embodiments, it is to be understood that it is not limited thereto. As will be apparent to those skilled in the art, numerous modifications and variations of these embodiments may be made without departing from the spirit of the invention or the scope of the following claims.

30 The embodiments of the invention in which an exclusive property or privilege is claimed are defined as follows:

1. A poly(hexafluoropropylene oxide) oil composition which comprises, as the base, a major amount of poly(hexafluoropropylene oxide) oil of the formula



or



where  $n$ ,  $p$  and  $r$  are integers indicating the degree of polymerization and  $R_f$  is a perfluoroalkyl group having 1 to 6 carbon atoms, said oil having an average molecular weight of at least 3,000 and a pour point not in excess of 50° F. and, as rust inhibitor, an effective amount of perfluoroalkylether compound selected from the group consisting of acids and corresponding ammonium salts of the formula



in which  $m$  is 7 to 10, B is H or  $NH_4$  and  $R_f$  is as previously stated.

2. The composition of claim 1 in which the poly(hexafluoropropylene oxide) oil is of the formula



and 0.1 to 2% by weight of perfluoroalkylether acid is present.

3. The composition of claim 2 in which  $R_f$  is



the poly(hexafluoropropylene oxide) oil has an average molecular weight of 5,500 to 7,000 and 1 to 2% of perfluoroalkylether acid is present.

65 4. The composition of claim 1 in which the poly(hexafluoropropylene oxide) oil is of the formula



and 0.1 to 2% by weight of the ammonium salt of perfluoroalkylether acid is present.

70 5. The composition of claim 4 in which  $R_f$  is



the poly(hexafluoropropylene oxide) oil has an average molecular weight of 5,500 to 7,000 and 1 to 2% of the

ammonium salt of perfluoroalkylether acid is present.  
 6. The composition of claim 1 in which the poly(hexafluoropropylene oxide) oil is of the formula



5 and 0.1 to 2% by weight of perfluoroalkylether acid is present.

7. The composition of claim 6 in which  $R_f$  is



10

the poly(hexafluoropropylene oxide) oil has an average molecular weight of 5,500 to 7,000 and 1 to 2% of perfluoroalkylether acid is present.

8. The composition of claim 1 in which the poly(hexafluoropropylene oxide) oil is of the formula



and 0.1 to 2% by weight of ammonium salt of perfluoroalkylether acid is present.

9. The composition of claim 8 in which  $R_f$  is



5 the poly(hexafluoropropylene oxide) oil has an average molecular weight of 5,500 to 7,000 and 1 to 2% of the ammonium salt of perfluoroalkylether acid is present.

#### References Cited

##### UNITED STATES PATENTS

3,242,218 3/1966 Miller ----- 260—535

15 DANIEL E. WYMAN, Primary Examiner

W. H. CANNON, Assistant Examiner.